

J. H. YOUNG,  
PROTECTED METAL ARTICLE,  
APPLICATION FILED MAR. 26, 1921.

1,418,347.

Patented June 6, 1922.



Inventor:  
James Howard Young  
By  
Jas. A. Chisholm, atty.

# UNITED STATES PATENT OFFICE.

JAMES HOWARD YOUNG, OF PITTSBURGH, PENNSYLVANIA, ASSIGNOR TO H. H. ROBERTSON COMPANY, OF PITTSBURGH, PENNSYLVANIA, A CORPORATION OF PENNSYLVANIA.

## PROTECTED METAL ARTICLE.

1,418,347.

Specification of Letters Patent. Patented June 6, 1922.

Application filed March 26, 1921. Serial No. 455,967.

*To all whom it may concern:*

Be it known that I, JAMES HOWARD YOUNG, a citizen of the United States, residing in Pittsburgh, in the county of Allegheny and State of Pennsylvania, have invented an Improvement in Protected Metal Articles, of which the following description, in connection with the accompanying drawings, is a specification like characters on the drawings representing like parts.

This invention relates to a protected metal article of that character in which an article of corrodible metal, such as iron or steel, is protected against corrosion by a layer of asphalt or like bituminous material alone or in conjunction with layers of fibrous material, such as asbestos, wool, or other fibrous felts.

Protective metal articles of the character described are efficient against corrosion as long as the bituminous layer remains intact, but where the bituminous layer is exposed, it is subject to the deleterious action of light, heat, and atmospheric conditions; also to abrasion and other mechanical actions in handling, crating and shipping, and in some cases to injury by adhesion of one protected article to another.

The present invention has for its object to provide a protected metal article of the character described, which possesses all of the advantageous features of the protected articles above referred to, and in addition possesses highly desirable features not possessed by them, among which may be mentioned, high light and heat reflecting properties, which enable the protected article to be effectively used in warm climates, as well as in cold climates, and which can be given any surface color desired with any drying oil paints. Also the detrimental effects of abrasion and other mechanical actions as well as adhesion are avoided.

To this end, an iron or steel article, either rigid or flexible and in any shape or form, which is provided with an exposed layer of asphalt, bitumen or like hydrocarbonaceous material, is provided with a relatively thin substantially non-corrodible metallic layer which is adhesively affixed to the corrodible metal article by the interposed layer of hydrocarbonaceous material.

The layer of relatively non-corrodible metal may consist of finely divided metals,

which have high light and heat reflecting properties, as will be described.

These and other features of this invention will be pointed out in the claims at the end of this specification.

Fig. 1 is a plan view of one form of protected metal article embodying this invention, and

Fig. 2, a section on an enlarged scale on the line 2—2, Fig. 1.

Referring to the drawing, *a* represents an article of corrodible metal, such as iron or steel, which may be rigid or flexible and of any form, and which is herein represented as a metal sheet.

The metal article *a* is provided with a protective layer *b* of asphalt or hydrocarbonaceous material of like character, which may be applied in any suitable manner as by passing the article *a* through a bath of melted asphalt, and to the layer *b* is applied layers *c* of asbestos, wool or other fibrous felt, which is provided with a layer *d* of asphalt or like hydrocarbonaceous material. The protected metal article thus described is provided with an outer surface of asphalt or like hydrocarbonaceous material, which is black or dark colored and open to the objections inherent in asphalt and like hydrocarbonaceous materials.

In accordance with the present invention, the protected article is provided with a relatively thin flexible layer *e* of substantially or relatively non-corrodible light colored metal, preferably aluminum, but which may be copper, zinc or other well-known pigments used in the so-called bronzing liquids. These pigments may be applied to the bituminous surfaces while the latter are hot and tacky and in condition to permit the pigments being firmly embedded in the same, or as may be preferred, the pigments may be applied in the form of a paint, in which case, the paint is provided with a vehicle for the pigment which exerts no appreciable solvent action on the bituminous surface and which when dry forms a firm, elastic, weather-resisting film, which is not tacky, and which is a good light and heat reflector.

A suitable paint for this purpose may be made by employing cellulose nitrate or acetate as a binder for the finely divided relatively non-corrodible metal, preferably aluminum, and using a solvent for the cellulose

compounds, which is volatile and practically inactive on asphalt or like hydrocarbonaceous material. A suitable solvent may be obtained by mixing about 20% acetone with about 20% glacial acetic acid and about 55% ethyl alcohol. If desired a suitable softening agent such as castor oil may be added to the paint.

The aluminum or other light colored non-corrodible metal in a finely divided condition is bound together by the cellulose nitrate or acetate binder and is present in sufficient quantity in the paint, to thoroughly cover the bituminous layer to which it is applied and thoroughly and effectively protect the same against the extraneous influences of the atmosphere, gases and fumes, and effectively seals the volatile constituents of the bituminous layer, thereby prolonging the protective value of said layer, and in addition reflects light and heat so efficiently as to enable the protected metal article to be used in warm climates as well as in the cooler or cold climates.

Furthermore the bright metallic exterior layer affords protection for the bituminous layer against abrasion, and avoids sticking of contiguous articles, thus facilitating packing, crating and transportation.

So also the bright metal exterior surface for the protected metal article, enables the latter to be painted with a drying oil paint of any desired color.

I have herein described one construction of protected metal article in which fibrous layers are used, but it is not desired to limit the invention in this respect.

Claims:

1. As an improved article of manufacture, a protected metal article comprising an article of corrodible metal, a layer of bitu-

minous or like hydrocarbonaceous material covering said corrodible metal, and a layer of finely divided relatively non-corrodible metal adhesively affixed to said hydrocarbonaceous material.

2. As an improved article of manufacture, a protected metal article comprising an article of corrodible metal, a layer of bituminous or like hydrocarbonaceous material covering said corrodible metal, and a layer of relatively non-corrodible metal adhesively affixed to said hydrocarbonaceous layer and composed of finely divided light colored relatively non-corrodible metal united by a binder of cellulose derivative.

3. As an improved article of manufacture, a protected metal article comprising an article of corrodible metal, a layer of bituminous or like hydrocarbonaceous material covering said corrodible metal, and a relatively thin layer of relatively non-corrodible metal adhesively affixed to the corrodible metal article by said hydrocarbonaceous layer.

4. As an improved article of manufacture, a protected metal article comprising an article of corrodible metal, a layer of bituminous or like hydrocarbonaceous material covering said corrodible metal, and a layer metallic in appearance and consisting of a cellulose derivative and comminuted material metallic in appearance.

5. An article having applied thereto a layer of bituminous or like hydrocarbonaceous material and an insoluble weather-resisting layer composed of a comminuted bright metal and a binder of cellulose.

In testimony whereof, I have signed my name to this specification.

JAMES HOWARD YOUNG.